

# UNITED STATES PATENT OFFICE.

FRANÇOIS AUGUSTE ROUX, OF PARIS, FRANCE, ASSIGNOR TO SOCIÉTÉ L'ALUMINIUM  
FRANCAIS, OF PARIS, FRANCE.

## TREATMENT OF SURFACES OF ALUMINUM OR ALLOYS OF ALUMINUM IN ORDER TO PREPARE THEM FOR RECEIVING A METALLIC DEPOSIT.

1,144,000.

Specification of Letters Patent. Patented June 22, 1915.

No Drawing.

Application filed January 19, 1914. Serial No. 813,062.

*To all whom it may concern:*

Be it known that I, FRANÇOIS AUGUSTE ROUX, a citizen of the Republic of France, and resident of Paris, France, have invented 5 new and useful improvements relating to the treatment of surfaces of aluminum or alloys of aluminum in order to prepare them for receiving a metallic deposit, which are fully set forth in the following specification.

- 10 When it is required to coat aluminum with metals by electrolytic action, and if, before this operation is carried out, the necessary pickling or cleansing is performed, it is observed that all the cleansing agents 15 which are known leave on the surface of aluminum a thin film of oxid and a shell or cover of hydrogen, the said film and cover preventing the adherence of the metals to be deposited on the said surface. To overcome 20 this difficulty various methods have already been proposed. One of the processes consists in submitting aluminum to the action of baths which precipitate, on its surface, heavy metals having for object to prevent 25 its oxidation. According to another method, and with the same end in view, a solution of a neutral metallic fluorid is employed in a neutral alkaline salt derived from an organic acid. It is also possible to bring consecutively into action both the solutions, by 30 beginning with the first named. However these processes have the disadvantage of leaving on the aluminum, at the moment when it is introduced into the galvanic 35 baths, a pulverulent deposit which a rinsing and even a brushing are not able to remove, and which a passage through an acid bath would wholly eliminate, leaving the oxidized metal bare. In such instance, perfect adherence of the metals to be deposited is impossible. If placed into the baths with the 40 pulverulent deposit, the deposits are rough and lend themselves poorly to polishing, and at the same time they are liable to disappear 45 at certain points in the electrolytic baths, from which there results an incomplete adherence of the deposited metal.

The present process consists in submitting the aluminum surfaces, previously cleansed 50 by any known means, to the action of diluted hydracids or of diluted alkalis, to which has

been added a salt of tin or of another soluble metal; then, after rinsing, the said surfaces are passed through a salt solution that is capable of fixing on them the tin or other 55 metal and at the same time of expelling the hydrogen which was inclosed in the pulverulent metallic deposit formed on the aluminum. The aluminum salts and the alums in a saturated and more or less warm solution 60 realize particularly well this latter condition, all the more as they have the property of dissolving the metallic oxids, which is 65 very advantageous for the performing of the process.

In carrying out the present invention, the aluminum surface to be coated is cleansed by any method, for instance by a solution of soda or potash at about 5%, which is preferably employed when hot; then the last traces 70 of alkali are washed away or neutralized, if necessary, in a bath of diluted sulfuric or nitric acid, or in a mixture of both these acids; after that, the metal, having first been thoroughly rinsed in water, is immersed in 75 a diluted solution of a hydracid or an alkaline hydrate at about 5 degrees Baumé, to which is added a salt of tin or of another soluble metal. For instance tin chlorid in the proportion of 1% gives good results. 80 The articles are then quickly and thoroughly rinsed, after which they are immersed into a saturated solution, preferably in a heated state, of an aluminum salt. Ammonia alum is especially to be recommended. During 85 the operation the hydrogen inclosed in the layer of soluble metal deposited on the aluminum escapes violently and at the same time it removes mechanically the pulverulent deposit which is in excess, it prevents 90 the oxidation of aluminum and gives tenacity to the tin or heavy metal deposit. The aluminum after having been so treated is then rinsed, and subsequently immersed in a solution of a diluted mineral acid—sulfuric 95 or nitric—the effect thereof consisting in dissolving the last traces of the metallic precipitate of which the adherence would not be sufficient to offer a proper resistance to the electrolytic baths. The latter operation 100 is not absolutely indispensable. Having been rinsed, the aluminum is ready to receive

all electrolytic deposits. It also may be kept in abeyance in pure water, or it may be dried. In any case its surface will not become oxidized and will always remain fit to receive a metallic deposit.

What I claim is:

1. A process of treating surfaces of aluminum or its alloys to prepare them for receiving a metallic deposit, which consists in subjecting the previously cleansed surfaces to the action of a weak bath containing a hydacid holding a soluble metal in solution, thereby to precipitate a deposit of said soluble metal upon said surfaces and to liberate hydrogen which remains occluded in the deposit where it adheres to said surfaces, rinsing said surfaces, and passing the surfaces through a hot bath constituted by a saturated solution of a salt capable of expelling the occluded hydrogen and of fixing on said surfaces the soluble metal employed.
2. A process of treating surfaces of aluminum or its alloys to prepare them for receiving a metallic deposit, which consists in subjecting the previously cleansed surfaces to the action of a weak bath containing a hydacid holding tin in solution, thereby to precipitate a deposit of tin upon said surfaces and to liberate hydrogen which remains occluded in the deposit where it adheres to said surfaces, rinsing said surfaces, and passing the surfaces through a hot bath constituted by a saturated solution of a salt capable of expelling the occluded hydrogen and of fixing the tin on said surfaces.
3. A process of treating surfaces of aluminum or its alloys to prepare them for receiving a metallic deposit, which consists in subjecting the previously cleansed surfaces to the action of a weak bath containing a hydacid holding tin in solution, rinsing said surfaces, and passing them through a

hot bath constituted by a saturated solution of an aluminum salt.

4. A process of treating surfaces of aluminum or its alloys to prepare them for receiving a metallic deposit, which consists in subjecting the previously cleansed surfaces to the action of a weak bath containing a substance holding a soluble metal in solution, thereby to precipitate a deposit of said soluble metal upon said surfaces and to liberate hydrogen which remains occluded in the deposit where it adheres to said surfaces, rinsing said surfaces, and passing the surfaces through a hot bath constituted by a saturated solution of a salt capable of expelling the occluded hydrogen and of fixing on said surfaces the soluble metal employed.

5. A process of treating surfaces of aluminum or its alloys to prepare them for receiving a metallic deposit, which consists in subjecting the previously cleansed surfaces to the action of a weak bath containing a hydacid holding a soluble metal in solution, thereby to precipitate a deposit of said soluble metal upon said surfaces and to liberate hydrogen which remains occluded in the deposit where it adheres to said surfaces, rinsing said surfaces, passing the surfaces through a hot bath constituted by a saturated solution of a salt capable of expelling the occluded hydrogen and of fixing on said surfaces the soluble metal employed, and immersing said surfaces in a mineral acid solution.

In testimony whereof I have signed this specification in the presence of two subscribing witnesses.

FRANÇOIS AUGUSTE ROUX.

Witnesses:

EMILE LEDRET,  
HANSON C. COXE.